

## UNITED STATES PATENT OFFICE

2,240,609

MINERAL OIL COMPOSITION AND  
IMPROVING AGENTDarwin E. Badertscher, Woodbury, N. J., assignor  
to Socony-Vacuum Oil Company, Incorporated,  
New York, N. Y., a corporation of New YorkNo Drawing. Application May 26, 1939,  
Serial No. 275,853

12 Claims. (Cl. 252—47)

This invention has to do in a general way with viscous mineral oil compositions and is more particularly concerned with the improvement of various properties of viscous mineral oil fractions refined for various uses, such improvement being effected by the addition thereto of a novel improving agent.

More specifically, one phase of this invention contemplates the stabilization of viscous mineral oil fractions against the harmful effects of oxidation. Another phase of the invention contemplates improvement of the load-carrying capacity of mineral oil fractions refined for use under extreme pressure conditions. This invention also contemplates novel oil-improving agents which may be used with viscous mineral oil fractions under various conditions of use to effect the improvement or improvements noted above.

As is well known to those familiar with the art, substantially all the various fractions obtained from mineral oils and refined for their various uses are susceptible to oxidation. The susceptibility of an oil fraction to oxidation and the manner in which oxidation manifests itself within the oil varies with the type and degree of refinement to which the oil has been subjected and with the conditions under which it is used or tested. In other words, the products formed in an oil fraction as a result of oxidation and the degree to which they are formed depends upon the extent to which the various unstable constituents or constituents which may act as oxidation catalysts have been removed by refining operations, and also upon the conditions of use.

A "highly refined" viscous oil, for example, which is one that has been refined by treatment with fuming sulfuric acid or other means or combinations such as  $AlCl_3$ , solvents and acids (or with large quantities of concentrated sulfuric acid), tends to form relatively large amounts of acidic constituents when subjected to oxidizing conditions. The presence of catalytic materials such as copper does not appear to affect appreciably the oxidation of highly refined oils, and such oils are less prone to the formation of colored bodies or of insoluble sludge. The formation of acidic bodies, however, is highly undesirable for most applications of these oils. For example, when used as an insulating or cooling oil in electrical equipment such as transformers or capacitors an increase in acidic bodies tends to lower the dielectric strength of the oil and has other harmful effects which are

undesirable. The acids are corrosive to metals and thus reduce the useful life of the oils as lubricants or for other purposes in which they come in contact with metals, and the acidic materials are also injurious in textile lubricants and in spray oils.

"Moderately refined" oils, which are normally oils that have been refined by treatment with only moderate amounts of sulfuric acid, or other refining agents, tend to form relatively small amounts of acidic oxidation products as compared with highly refined oils, but they undergo material color depreciation and form considerable amounts of sludge. The changes taking place in these oils are appreciably accelerated by the presence of metal catalysts such as copper. Sufficient acid is generally formed to cause some reduction in the dielectric strength of these oils, but the principal objection to them is their tendency to deposit sludge which interferes with heat transfer in transformers and turbines and also causes plugging of oil feed lines in lubricating systems.

"Solvent-refined" oils in general, which are normally prepared by treatment with selective solvents, such as chlorex, phenol, furfural, etc., resemble the moderately refined acid-treated oils in that their oxidation is accelerated by the presence of metals such as copper and further in that it is attended by substantial color depreciation and sludge formation. Acid formation is usually greater than in the case of moderately acid-refined oils, but considerably less than with highly refined oils. Both sludge and acid formation lower their value for many purposes, such as electrical insulation, lubrication, etc. Also solvent-refined oils have found extensive use as lubricants for internal combustion engines because of their high viscosity index, but under the conditions of use encountered in crankcases such oils develop constituents which are corrosive toward certain metal bearings such as cadmium-silver bearings, etc., which are sometimes used.

It is to be understood that this classification of oils as "highly refined," "moderately refined" and "solvent-refined" is by no means limiting and that there can exist oils whose refining and blending has been such as to make them intermediate in properties between the types set up. Thus, response to inhibitors may be said to depend entirely upon the type of oxidation and end products of oxidation of an oil, which in turn depends largely upon the degree of refining this oil has had. Further, the degree of refining re-

quired to produce these types of oils varies with the crude source so that any one refining procedure may produce either a highly refined oil or a moderately refined oil, depending upon the crude source. Pennsylvania type oils, for example, require much less refining to produce highly refined oils than the Coastal type of oils.

The use of oxidation inhibitors for the purpose of stabilizing a viscous mineral oil fraction against the deleterious effects of oxidation discussed above is well known. Since the action of these inhibiting materials is apparently catalytic, the problem of their development is a difficult one and is evidently influenced to a large degree by the oxidizable constituents which are in the oil following a particular refining treatment. Thus, a particular inhibitor or class of inhibitors may be effective to stabilize a highly refined oil against acid formation while the same inhibitor may have no appreciable effect upon acid, color or sludge formation in a moderately refined oil and vice versa. The same inhibitor may or may not be effective in inhibiting acid, sludge and color formation in a solvent-refined oil and may or may not be effective to inhibit the corrosive action of a solvent-refined oil toward metals such, for example, as the various normally corroded alloys typified by cadmium-silver bearings.

The compounds of the present invention are particularly useful as inhibitors of acid formation in highly refined oils, inhibitors of bearing corrosion in solvent-refined motor oils under conditions of crankcase use, and also as extreme pressure bases in lubricants of the type used in hypoid gears, etc. The tests which I have conducted indicate that these compounds do not show appreciable effect toward the inhibition of the deleterious effects of oxidation upon moderately refined mineral oil fractions of the turbine oil type.

Although this invention is broadly concerned with any viscous mineral oil fraction containing an improving agent falling into the class of novel compounds contemplated herein, it is more specifically concerned with the stabilization of the so-called highly refined oils against acid formation, the stabilization of moderately refined oils against alloy bearing corrosion and the improvement of the load-carrying capacity of lubricating oils of the extreme pressure type.

The compounds contemplated herein as oil-improving agents are obtained by the reaction of an alkali alkyl xanthate on a beta-chloroethyl amine. The products obtained by such reaction cannot be classified with certainty as definite chemical compounds and are therefore referred to and defined herein merely as products of the reaction generally described above. The general procedure followed in effecting this reaction is to employ substantially equivalent proportions of the alkali alkyl xanthate and the beta-chloroethyl amine, such compounds being admixed with a suitable liquid medium, such as ethyl alcohol, and refluxed for a substantial period of time, during which the compounds react with the release of an alkali chloride. The alkali chloride is separated from the reaction product in any suitable manner, such as by filtration, and the reaction product is subjected to purification which will be described in greater detail later on.

Although, as indicated above, I do not wish to be bound by any theory as to what reaction takes place or as to what the chemical composition of the reaction product is, it does appear from the

reactants used and the sulfur and nitrogen content of the reaction product that when an alkali alkyl xanthate is reacted with a tris(beta-chloroethyl) amine, the reaction takes place according to the following equation:



in which R indicates an alkyl group such as ethyl, propyl, butyl, amyl, etc., and M indicates an alkali metal such as potassium or sodium.

Further illustrating the preparation of the reaction products contemplated herein as oil-improving agents an exemplary product was prepared from potassium butyl xanthate and tris(beta-chloroethyl) amine according to the following procedure:

A mixture of 12 grams of tris(beta-chloroethyl) amine, 39 grams of potassium butyl xanthate, and 200 cc. of a suitable solvent such as 95 per cent ethyl alcohol was stirred and refluxed for a period of 5 hours. The white solid potassium chloride which had been separated was filtered off and washed with hot alcohol. A yellow lower layer formed in the filtrate and was separated from the alcohol, the alcohol layer being drowned in water and the separated material being extracted twice with benzene and twice with ethyl ether. The original yellow lower layer was combined with the extract and filtered and distilled to remove the solvent. This procedure yielded 20 grams of residue of pale yellow oil which analyzed without further purification 2.77 per cent nitrogen and 35.2 per cent sulfur. On the basis of an assumed composition,  $C_{21}H_{39}O_3S_6N$ , which in the equation above would be



40 the nitrogen content would be 2.57 per cent and the sulfur content 35.2 per cent.

The following examples illustrate the effectiveness of a compound or reaction product obtained according to the foregoing procedure as an improving agent for representative types of mineral oils.

#### EXAMPLE I

##### (HIGHLY REFINED OILS)

The oil employed in this test was of the "highly refined" type used in transformers and the like which had been obtained from a Coastal distillate by successive treatments with 98 per cent sulfuric acid in the ratio of 40 pounds per barrel and 103 per cent oleum in the ratio of 180 pounds per barrel, followed by neutralization, washing, and clay percolation. The refined oil had a specific gravity of 0.871 and a flash point of 310° F. and a Saybolt Universal viscosity of 69 seconds at 100° F. It was tested by heating a 150 gram sample of the oil or the oil blend to 120° C. and bubbling oxygen gas therethrough for a period of 70 hours. The amount of acidic oxidation products thus formed in the oil was determined by titration with standard alkali and the results recorded in terms of neutralization number (N. N.), which represents the number of milligrams of KOH required to neutralize the acids formed in one gram of oil. The results of this test are set forth in Table I below, in which it will be observed that the reaction product contemplated by this invention was effective to inhibit to a substantial degree the acid formation in this highly refined oil.

Table I

|                                                                                                | Neutralization No.<br>after test |
|------------------------------------------------------------------------------------------------|----------------------------------|
| Oil alone                                                                                      | 25.0                             |
| Oil+0.10% of tris (beta-chloroethyl) amine<br>and potassium butyl xanthate reaction<br>product | 0.29                             |

## EXAMPLE II

## (SOLVENT-REFINED MOTOR OIL)

The oil used in this test was an S. A. E. 20 motor oil obtained from a Pennsylvania mixed neutral residuum stock by solvent-extraction with Chlorex. It had a specific gravity of 0.87, a flash point of 435° F. and a S. U. viscosity of 318 seconds at 100° F. The test used comprised passing a current of air at the rate of 2000 mls. per hour through a 50 ml. sample of the oil heated to a temperature of 347° F. for a period of 22 hours in the presence of a 6-gram section taken from a cadmium-silver bearing. The weight loss in milligrams was interpreted as a measure of the corrosiveness of the oil or oil blend and the results of this test using the oil alone and the same oil containing 0.25 per cent of the reaction product described above are given in Table II below.

Table II

|                                                                                               | Weight loss (mgs.) |    |
|-----------------------------------------------------------------------------------------------|--------------------|----|
| Oil alone                                                                                     | 95.0               | 30 |
| Oil+0.25% of tris (beta-chloroethyl) amine<br>and potassium butylxanthate reaction<br>product | 1.0                |    |

## EXAMPLE III

As has been previously pointed out, the reaction products contemplated by this invention also possess the property of improving the load-carrying capacity of lubricants designed for use under extreme pressure conditions as, for example, in the lubrication of hypoid gears and the like. The extreme pressure properties of these reaction products was demonstrated by a conventional extreme pressure test known as the S. A. E. test, in which the oil alone failed at a load of 15 pounds, whereas an oil blend containing 10 per cent of the reaction product described above passed the test at a load of 580 pounds at 750 R. P. M.

It is to be understood that reaction products of the type contemplated by this invention can be used in the oil in various proportions, depending upon the oil fraction to which they are added and the particular properties which it is desired to improve. In general it appears that the range of proportions, taking in both the oxidation-inhibitive action and the extreme pressure action, will be from about 0.05 per cent to about 15 per cent.

It is also to be understood that the terms "highly refined" and "solvent-refined" as used herein are not necessarily restricted to a particular refining treatment but have reference to oils or oil fractions corresponding substantially in their manner of deterioration and inhibitor response to the examples given. As has been previously pointed out, the final characteristics of a mineral oil fraction are affected by the crude oil from which such fraction is obtained, as well as by the refining treatment to which it has been subjected. It is possible, for example, by the choice of a particular crude to obtain a highly refined oil with a refining treatment which when applied to another crude would yield an oil of the moderately refined type.

## I claim:

1. A mineral oil composition comprising a viscous mineral oil fraction having in admixture therewith a minor proportion of the reaction product obtained by dissolving substantially equivalent proportions of an alkali alkyl xanthate and a beta-chloroethyl amine in a suitable solvent medium; refluxing the mixture for a sufficient period of time to precipitate alkali chloride and form the reaction product; and removing the alkali chloride and the solvent from said reaction product.
2. A mineral oil composition comprising a viscous mineral oil fraction having in admixture therewith a minor proportion of the reaction product obtained by dissolving substantially equivalent proportions of potassium butyl xanthate and tris(beta-chloroethyl) amine in a suitable solvent medium; refluxing the mixture for a sufficient period of time to precipitate potassium chloride and form the reaction product; and removing the potassium chloride and the solvent from said reaction product.
3. A mineral oil composition comprising a viscous mineral oil fraction selected from the group consisting of highly refined viscous oils and solvent-refined motor oils having in admixture therewith a minor proportion of the reaction product obtained by dissolving substantially equivalent proportions of an alkali alkyl xanthate and a beta-chloroethyl amine in a suitable solvent medium; refluxing the mixture for a sufficient period of time to precipitate alkali chloride and form the reaction product; and removing the alkali chloride and the solvent from said reaction product.
4. An extreme pressure lubricant composition comprising a major proportion of mineral lubricating oil and a minor proportion of the reaction product obtained by dissolving substantially equivalent proportions of an alkali alkyl xanthate and a beta-chloroethyl amine in a suitable solvent medium; refluxing the mixture for a sufficient period of time to precipitate alkali chloride and form the reaction product; and removing the alkali chloride and the solvent from said reaction product.
5. A mineral oil composition comprising a viscous mineral oil fraction selected from the group consisting of highly refined viscous oils and solvent-refined motor oils having in admixture therewith a minor proportion of the reaction product obtained by dissolving substantially equivalent proportions of potassium butyl xanthate and tris(beta-chloroethyl) amine in a suitable solvent medium; refluxing the mixture for a sufficient period of time to precipitate potassium chloride and form the reaction product; and removing the potassium chloride and the solvent from said reaction product.
6. An extreme pressure lubricant composition comprising a major proportion of mineral lubricating oil and a minor proportion of the reaction product obtained by dissolving substantially equivalent proportions of potassium butyl xanthate and tris(beta-chloroethyl) amine in a suitable solvent medium; refluxing the mixture for a sufficient period of time to precipitate potassium chloride and form the reaction product; and removing the potassium chloride and the solvent from the reaction product.
7. A mineral oil composition comprising a viscous mineral oil fraction having in admixture therewith a minor proportion of the reaction product obtained by reacting together under re-

flux in a suitable solvent about three molecular proportions of an alkali alkyl xanthate and about one molecular proportion of tris(beta-chloroethyl) amine for a sufficient period of time to precipitate an alkali chloride and form the reaction product, and separating the alkali chloride and the solvent from the reaction product.

8. A mineral oil composition comprising a viscous mineral oil fraction having in admixture therewith from about 0.05% to about 15% of the reaction product obtained by reacting together under reflux in a suitable solvent substantially equivalent proportions of an alkali alkyl xanthate and a beta-chloroethyl amine for a sufficient period of time to precipitate an alkali chloride and form the reaction product, and separating the alkali chloride and the solvent from the said reaction product.

9. A mineral oil composition comprising a viscous mineral oil fraction having in admixture therewith from about 0.05% to about 15% of the reaction product obtained by reacting together under reflux in a suitable solvent about three molecular proportions of an alkali alkyl xanthate and about one molecular proportion of tris(beta-chloroethyl) amine for a sufficient period of time to precipitate an alkali chloride and form the reaction product, and separating the alkali chloride and the solvent from the reaction product.

10. A mineral oil improving agent comprising the product obtained by reacting together under reflux in a suitable solvent substantially equivalent proportions of an alkali alkyl xanthate and a beta-chloroethyl amine for a sufficient period of time to precipitate alkali-chloride and form the reaction product and separating the alkali chloride and the solvent from the said reaction product.

11. A mineral oil improving agent comprising the product obtained by reacting together under reflux in a suitable solvent about three molecular proportions of an alkali alkyl xanthate and about one molecular proportion of tris(beta-chloroethyl) amine for a sufficient period of time to precipitate alkali chloride and form the reaction product, and separating the alkali chloride and the solvent from the said reaction product.

12. A mineral oil improving agent comprising the product obtained by reacting together under reflux in a suitable solvent about three molecular proportions of potassium butyl xanthate and about one molecular proportion of tris(beta-chloroethyl) amine for a sufficient time to precipitate potassium chloride and form the reaction product and separating the potassium chloride and the solvent from the said reaction product.

DARWIN E. BADERTSCHER.